

Feb. 23, 1932.

L. NORDENFELT

1,847,019

MANUFACTURE OF HOLLOW METAL BARS

Filed June 25, 1930

*Fig. 1.*



*Fig. 2.*



*Fig. 3.*



INVENTOR.  
*L. Nordenfelt*  
BY: *Marks & Clerk*  
ATTORNEYS.

## UNITED STATES PATENT OFFICE

LENNART NORDENFELT, OF HOFORS, SWEDEN

MANUFACTURE OF HOLLOW METAL BARS

Application filed June 25, 1930, Serial No. 463,835, and in Sweden June 28, 1929.

The present invention relates to a process of manufacturing hollow metal bars or tubes, for instance mining drills, boiler stay-bolts, from hollow billets or ingots, and, more particularly, the invention relates to an improvement of the process consisting therein that a core is inserted into a hole in the blank. The blank then is rolled, forged or stretched in order to receive the shape aimed at, and, to allow the core to be removed from the finished object, said core then being exposed to a stretching operation so as to reduce its diameter.

In processes, hitherto known and based upon this principle, the last mentioned operation, viz. the stretching of the core and its removing from the object, has presented great difficulties, as the core material used, viz. common steel or forgeable iron, at the stretching operation is exposed only to local contractions, and even if the stretching process has been carried to the stress of ultimate tenacity, considerable portions of the core still present the same diameter as the inner diameter of the hole made in the blank, and offer a great resistance to the removal of the core, thus making the work more expensive. The appearance of local contractions depends on the presence of a strong friction between the core and the walls of the hole.

If this friction is not overcome a contraction evenly distributed along the whole length of the core will not take place, on the contrary the core at the stretching operation will be lengthened at the two points where a groove has been made in the ready-made blank and where no local friction thus is to be found. Thus, the stretching takes place along a very short portion of the core's length, and when the local contraction and fracture occur, the remaining part of the core will remain in the blank practically without any reduction of its diameter. In order to obviate this inconvenience it has been suggested to use a metal or metal alloy as core ma-

terial which, at the stretching operation, is lengthened essentially uniformly along its entire length and thereby obtains a uniform reduction of its diameter. Such a core material must have a strength tenacity greater than the resistance caused by friction between the core and the walls of the hole. In such a case the resistance, due to friction, will positively be overcome, and the evenly distributed extension and thus also the contraction are free to take place along the whole length of the core. Thus, the core, after the stretching operation, may safely be removed from the metal bar as a whole.

According to the present invention a process is suggested by means of which the resistance due to friction between the core and the metal bar at the stretching of the core is highly reduced so that core materials, also having a low strength of ultimate tenacity may be used.

The invention is essentially characterized by the fact that the core from the beginning is made with a diameter shorter than that of the hole in the blank, so that the core will not fill it, and further thereby that the interspace, thus produced, is filled either by applying a suitable friction-reducing material round the core before inserting the latter into the hole of the blank or billet. When removing the core the lengthening properties of the core hereby will always be positively utilized and, owing thereto, the core may also be safely removed from the metal bar as a whole.

As examples of materials suitable to be inserted in order to reduce the resistance, due to friction between the core and the walls of the hole, sheets or strips of asbestos or similar material may be employed.

In the accompanying drawings:

Figure 1 is a perspective view showing a core being inserted into the hole of the billet.

Fig. 2 is a view showing a core in the act of being wrapped with the sheet material.

Fig. 3 is a view showing a core spirally wrapped with a strip of material.

Referring to the drawings, 1 designates the billet or blank and 2 the longitudinal holes therein. As shown in Fig. 1, the core 3 is wrapped with a sheet 4 of asbestos or other suitable material, the wrapping taking place before the core is inserted in the hole 2. In Fig. 3, in lieu of a sheet of material, a strip 5 of similar material is spirally wrapped around the core before insertion into the hole 2 of the billet.

It will thus be seen that the material is wrapped in a suitable manner round the core, which thereupon is introduced into the hole of the billet or blank. The rolling, forging or stretching then taking place so as to allow the blank to receive the desired shape. At this time, of course, as well the core inserted into the blank as the friction reducing material are given a corresponding deformation, and, generally, it is the matter of extending the blank while reducing its diameter.

The cross-section of the core and the cross-section of the friction reducing material are proportionally reduced, while the blank is brought to the desired shape. Owing to this fact a layer of the friction reducing material will always positively be obtained round the core in the blank.

The advantage arrived at by the invention now appears at the following operation, namely at the removing of the core which according to the present invention will be removed very easily.

On account of the friction between the core and the walls of the hole having in a very efficient manner been reduced to an order of magnitude far below the stress of ultimate tenacity of the core material, the core may very easily be removed only after a relatively inconsiderable stretching, this stretching operation positively causing an essentially uniform lengthening of the entire length of the core so as to allow the core diameter to obtain a uniform reduction, whereby the core will rest loosely in the bar at the end of the stretching operation.

Having now particularly described the nature of my invention and the manner of its operation, what I claim is:—

1. Process of making hollow metal bars from hollow billets which consists in wrapping a metal core with a sheet of friction reducing material, the core being of a diameter less than the hole of the billet, then inserting the wrapped core into the hole of the billet so that the wrapping will occupy the entire space between the core and wall of the billet hole, then elongating and reducing the cross sectional area of the billet, and then pulling the core and wrapping as a whole from the billet.

2. Process of making hollow metal bars from hollow billets which consists in spi-

rally wrapping upon a metal core, a strip of friction reducing material, the core being of a diameter less than the diameter of the hole, then inserting the core in the hole of the billet so that the wound strip will occupy the entire space between the core and wall of the hole of the billet then elongating and reducing the cross sectional area of the billet, and then pulling the core and wrapping as a whole from the billet.

In testimony whereof I have affixed my signature.

LENNART NORDENFELT.

80

85

90

95

100

105

110

115

120

125

130